

## 1

3,318,990

METHOD OF MANUFACTURING FLAT  
VISCOSE FIBERSYoichi Kajitani, Saito, Japan, assignor to Kurashiki Rayon  
Company Limited, Kurashiki, Japan, a corporation of  
JapanNo Drawing. Filed Aug. 12, 1963, Ser. No. 301,625  
Claims priority, application Japan, Aug. 18, 1962,  
37/35,829

3 Claims. (Cl. 264—187)

The present invention relates to a method of manufacturing tubular and flat viscose fibers having lustres and excellent flatness characterized in that a viscose having an ammonium chloride value of more than 16 containing 2-50% of water swelling high molecular substance based on the cellulose in the viscose, and 2-4% of alkali carbonate based on the viscose is spun into a spinning bath containing sulfuric acid and sulfates.

Viscose fibers have recently been used in large quantity for making paper and non-woven cloths. Ordinary viscose fibers, however, different from wooden fibers and bast fiber, are difficult to be fibrillized by beating and also the adhesion between fibers can not be developed by the action of heat and water so that it is difficult to produce papers from viscose fibers alone, and it is necessary to add some other binder.

In order to solve the above difficulties it has recently been proposed to manufacture hollow viscose fibers by adding a suitable foaming agent and by a special manufacturing condition and a paper can be manufactured by using such fibers without adding any other binder. The reason for the above is based on the consideration that the fibers can be tightly adhered with each other by flattening the configuration when they are wetted and formed to a thin layer and when the thin layers are dried, water existing between fibers and contained in its interior part is evaporated and each fiber is further brought together more intimately to cause "van der Waals" bond or hydrogen bond between cellulose molecules constituting the fiber, thereby providing papers of sufficient strength by the intermolecular bonding force. The hollow flat viscose fibers obtained by known processes require strict manufacturing control, and even then sufficiently flat viscose fibers are difficult to obtain. In general a paper of sufficient strength can not be obtained by using such fibers. Moreover when the monofilament denier becomes large the flatness becomes gradually worse and even when it is sufficiently flat the adhesion of fibers with each other becomes insufficient and the spacing between fibers prevents the intermolecular bonding force of cellulose to act between each fiber so that such fibers alone are difficult to make papers.

In heretofore known hollow flat viscose fibers, usually if monofilament denier is more than 3 denier the average length (average thickness) of short axis of the flat part becomes more than  $4\mu$ . The self adhering property between fibers is almost or perfectly lost and when the paper made of heretofore known hollow flat viscose fibers only, is wetted, the inter-fibrous binding force is lost and the fiber is dispersed into water.

According to the present invention, by making tubular flat viscose fibers containing water swelling high molecular substance the inter-fibrous binding force when paper is manufactured is increased so that the manufacturing conditions are not critical. The invention also provides fibers having excellent flat condition, luster and superior self-adhering property. Moreover the tubular flat viscose fibers obtained by the method of the invention enables manufacture of paper having sufficient strength without adding any other binder even when monofilament denier becomes larger and the average length (average thickness) of the short axis of the flat part becomes

## 2

comparatively large and can perfectly obviate the basic disadvantages of heretofore known hollow flat viscose fibers in which the self-adhering property and paper making possibility in the large denier filaments are lost. Further, the paper obtained by using the tubular flat viscose fibers obtained by the method of the invention only does not lose the inter-fibrous binding force when wetted again but maintains the configuration of paper.

The hollow flat viscose fibers manufactured by heretofore known process and papers manufactured by such fibers have luster but the paper manufactured by the tubular flat viscose fiber and the paper manufactured by the fiber of the present invention have superior luster, and by hot-pressing the wet paper when manufactured the similar effect can be developed without applying treatment with surface coating agent.

The "water swelling high molecular substances" in the present invention means, for instance, polyvinyl alcohol (abridged as PVA hereafter) which is swelled by water at room temperature but soluble in warm water or hot water and PVA derivatives, or hemi cellulose, methyl cellulose, ethyl cellulose, cyanoethyl cellulose, carboxymethyl cellulose, hydroxyethyl cellulose and the like so-called alkali soluble cellulose derivatives. The "tubular flat viscose fiber" in the invention means such fiber containing 2-25% of such water swelling high molecular substance and at least 60% of the total length of the fiber have tightly adhered inner surfaces without hollow portion and consists of a tubular flattened portion of which the long axis of the cross section of the fiber is at least 5 times that of the short axis. The content of the water swelling high molecular substance in the fiber depend on the kinds, object and fitness etc. of the fiber but usually desirable to be of 2 to 50% of the weight of regenerated cellulose in fiber, preferably 5 to 30%.

The fiber having good luster and self-adhesivity necessitates such condition that the internal surfaces of the tubular flattened portion are almost preferably adhered without gap and upper and rear surfaces are smooth and substantially parallel and also it has possibly large flatness and the long axis of the cross section of the fiber should have at least 5 times that of the short axis, preferably more than 10 times to several 10 times and moreover, the tubular flattened part should be at least 60% of total length of fiber and as the ratio increases the luster and self-adhesivity are improved enabling to more easily obtain a paper of thin, large splitting length and luster like cellophane. However, according to the purpose of using the fiber there is sometimes preferable to mix 20 to 30% of solid fiber. For instance, if it is desired to obtain a paper having high splitting strength it is better to mix solid fiber rather than to make paper with flat fiber only. The tubular flat fiber of the invention may be obtained by spinning a younger ripening degree viscose containing 2 to 50% (based on the cellulose in viscose) of water swelling high molecular substance and 2 to 4% (based on the produced viscose) of alkali carbonate and having an ammonium chloride value of more than 16 into a spinning bath containing sulfuric acid and sulfate. The water swelling high molecular substance and alkali carbonate may be added at any suitable stage of viscose process and also may be added simultaneously or separately. In case of water swelling high molecular substance such as PVA it is preferable to react it with carbon disulfite to provide PVA xanthate solution. It is not necessary to use special viscose composition but it is preferable to take younger age viscose in case of spinning and an ammonium chloride value of about 20 is suitable.

In spinning such viscose it is usual to use spinning bath consisting of sulfuric acid, sodium sulfate and zinc sulfate, yet in this case the existence of zinc sulfate is not always necessary and sodium sulfate may be substi-

uted by magnesium sulfate, aluminum sulfate in combination and the concentration of sulfate is preferably high in order to prevent the dissolving of water swelling high molecular substance in viscose and to obtain superior flat viscose fibers the temperature and acidity of spinning bath are preferably high.

The fibers obtainable by the method of the invention may be used, besides for making paper, for non-woven cloths or clothes, domestic purposes, wall papers and other fibers for building construction.

*Example 1*

PVA having polymerization degree 1,700 was dissolved in hot water and added with caustic soda and carbon disulfide and mixed by stirring at 20° C. for 90 minutes to xanthate PVA. The PVA xanthate solution thus obtained containing 8.5% PVA and 5% alkali is added with viscose made by a conventional process consisting of 8.5% cellulose and 5% alkali at a rate of 2:8 and then added hereto with 3% (based on the produced viscose mixture) of sodium carbonate and agitated to dissolve.

After filtered and defoamed, the solution having aging degree of 18 ammonium chloride value was spun through a nozzle having 3,000 holes, 0.065 mm. dia. into the pinning bath consisting of 12% sulfuric acid, 2.5% zinc sulfate and 25% sodium sulfate at 60° C. and the filament thus spun was stretched for 40% into a hot water bath and after taken up at a spinning speed of 50 m./min. it was cut to a length of 4 mm. By changing delivery quantity of viscose under this condition tubular flat fibers having monofilament of 0.7 denier, 1.0 denier, 2.5 denier, 5 denier and 8 denier were obtained.

For the sake of comparison a conventional solution of viscose having the composition of 8.5% of ordinary viscose cellulose and 5% of alkali added with 3% of sodium carbonate same as above example, without adding PVA xanthate solution, and spun under the same condition and prepared same tubular flat fibers having different deniers.

The conditions of flatness of each fiber is as shown in the next table.

| Monomfilament dr. | Kind of filament | Adhesion of internal surface | Short axis of cross section ( $\mu$ ) | Long axis of cross section ( $\mu$ ) | Long axis/short axis |
|-------------------|------------------|------------------------------|---------------------------------------|--------------------------------------|----------------------|
| 1.7               | The invention    | Good                         | 1.6                                   | 43                                   | 26.9                 |
|                   | Contrast         | do                           | 1.9                                   | 38                                   | 20.0                 |
| 2.5               | The invention    | do                           | 2.3                                   | 55                                   | 23.9                 |
|                   | Contrast         | do                           | 2.8                                   | 47                                   | 17.8                 |
| 5                 | The invention    | do                           | 3.0                                   | 58                                   | 19.4                 |
|                   | Contrast         | Somewhat no good             | 3.6                                   | 61                                   | 16.9                 |
| 1.5               | The invention    | Good                         | 6.2                                   | 71                                   | 11.5                 |
|                   | Contrast         | No good                      | 7.0                                   | 70                                   | 10.0                 |
| 2.5               | The invention    | Somewhat no good             | 8.8                                   | 93                                   | 10.6                 |
|                   | Contrast         | No good                      | 9.2                                   | 84                                   | 9.2                  |

The fiber prepared by the method of the invention is lightly adhered in the internal surface and has a greater flatness compared with a conventional fiber and moreover even if the monofilament denier becomes larger good flat fibers can be obtained. The fibers obtained by the method of the invention were dispersed in water each independently and thereafter without adding other binder paper is made according to the TAPPI process by manual working and the wet paper thus obtained was pressed and dried by a hot press with the pressure of 0.5 kg./cm.<sup>2</sup> and at a temperature of 100° C., then as the result, all papers obtained from the fibers of the mixed spun PVA of the invention showed sufficient strength and excellent surface luster.

On the other hand, in a flat fiber obtained from viscose without mixing with PVA, when monofilament denier is less than 2.5 a paper may be made but with the flat fiber of 5 denier and 8 denier no paper could be manufactured.

*Example 2*

When sodium xanthate (xanthogen acid soda) prepared by a conventional process is dissolved it is added,

besides caustic soda, 3.5% (based on the produced viscose) of sodium carbonate and 10% (based on cellulose) of carboxy methyl cellulose and agitated at 15° C. for 3 hours to dissolve and 8% of thus produced cellulose and viscose of 8% of all alkalis were spun at an ammonium chloride value 22 into the spinning solution same as in Example 1. The fiber coming out of the spinning solution was stretched for 50% into a bath of 1% sulfuric acid at 50° C., then wound up at a speed of 30 m./min. and cut to a length of 4 mm. The fiber had monofilament denier of 1.5 and flat tubular section having perfectly adhered inner surfaces and the short axis of its cross section of 2.5 $\mu$  and long axis of 56 $\mu$ . A paper was made by using this fiber by the same manner as in Example 1, having the weight 52.45 g./m.<sup>2</sup>, thickness 0.08 mm., breaking length 38 km. and tear factor 190.

The paper made of the flat tubular fibers obtained under the same condition as above from viscose not containing carboxy methyl cellulose showed the weight of 53.18 g./m.<sup>2</sup>, thickness of 0.12 mm., breaking length of 1.35 km. and tear factor 220. With fibers of the method of the invention a very thin paper was produced having a large breaking length.

In the specification and the claims, all percents are on a weight basis.

What I claim is:

1. A method of manufacturing tubular flat viscose fibers, which comprises spinning viscose having an aging degree represented by an ammonium chloride value of more than 16 to a spinning solution containing sulphuric acid and sulphate, said viscose containing 2 to 50%, based on the weight of cellulose in viscose, of a water swelling substance selected from the group consisting of polyvinyl alcohol, polyvinyl alcohol derivatives, and alkali soluble cellulose derivatives and containing 2 to 4%, based on the weight of viscose, of alkali carbonate, whereby tubular flat viscose fibers are obtained.

2. A method according to claim 1, wherein the water swelling substance is selected from the group consisting of hemi cellulose, methyl cellulose, ethyl cellulose, cyanoethyl cellulose, and hydroxyethyl cellulose.

3. A method according to claim 1, wherein the fiber is made from a sodium xanthate dissolved by addition of caustic soda, alkali carbonate and carboxy methyl cellulose.

**References Cited by the Examiner**

**UNITED STATES PATENTS**

|    |           |         |                   |           |           |
|----|-----------|---------|-------------------|-----------|-----------|
| 60 | 1,464,048 | 8/1923  | Rousset           | -----     | 161—178   |
|    | 2,085,513 | 6/1937  | Steindorff et al. | -----     | 106—164   |
|    | 2,162,460 | 6/1939  | Maxwell           |           |           |
|    | 2,165,393 | 7/1939  | Lilienfeld        | -----     | 106—164   |
|    | 2,176,085 | 10/1939 | Lilienfeld        | -----     | 106—164   |
| 65 | 2,201,663 | 5/1940  | Ellsworth et al.  |           |           |
|    | 2,265,915 | 12/1941 | Lilienfeld        |           |           |
|    | 2,267,217 | 12/1941 | Reichel           |           |           |
|    | 2,783,158 | 2/1957  | Entwistle et al.  |           |           |
| 70 | 2,796,656 | 6/1957  | Schappel et al.   | 264—198 X |           |
|    | 2,835,551 | 5/1958  | Kosuge            | -----     | 161—178 X |

**FOREIGN PATENTS**

37-5810 6/1962 Japan.

ALEXANDER H. BRODMERKEL, Primary Examiner.  
J. H. WOO, Assistant Examiner.